

Aug. 26, 1930.

G. P. McNIFF

1,773,741

METHOD OF MAKING PROJECTILES

Filed Dec. 7, 1925



WITNESS

J. G. Gahagan Bradley.

INVENTOR

Gilbert P. McNiff  
By Cleveland McCallister  
His attorney

## UNITED STATES PATENT OFFICE

GILBERT P. MCNIFF, OF PITTSBURGH, PENNSYLVANIA

## METHOD OF MAKING PROJECTILES

Application filed December 7, 1925. Serial No. 73,675.

This invention relates to projectiles or explosive shells such as are manufactured in various sizes to be fired from guns of different calibers; and it relates more particularly to the manufacture of shell forgings which are loaded with charges of powder, shrapnel or the like to form the finished projectiles. The latter as ordinarily manufactured comprise a body portion of streamline contour filled with an explosive adapted to be detonated by one of several detonators or fuses which are usually secured to and close the forward end or nose of the shell forging.

Shell forgings have heretofore been manufactured solely by the pierce and draw method in which a solid billet is pierced in a closed die by a hydraulic plunger so as to form a rough blank closed at one end. The great difficulty of machining and finishing a blank of this type results largely from the fact that, one end being closed, it is necessary to do all the inside machining and shaping from the other end of the blank. A separate machining operation from the boring of the interior diameter is also required to finish the inside of the base and care must be used to keep the thickness of the base within the required limits.

An object of this invention is to provide an improved and simplified method of manufacturing shell forgings.

The manufacture of projectiles by the pierce and draw method requires special machines, consequently under emergency conditions the capacity of this country to produce shell forgings by that method is limited by the capacity of such special machinery as there may then be in existence.

A further object of this invention is to provide a method of making shell forgings capable of being carried to completion by standard machines. Obviously such a method, permitting an immediate, high production of shell forgings with standard equipment has immeasurable advantages.

The shell produced by the pierce and draw method of manufacture is only about 80% efficient for destructive purposes for the reason that, upon explosion only about 80% of

the body breaks into fragments which are of the destructive size and shape, viz., the size of a pea or pebble. From 10% to 20% of the shell body is powdered or is broken into such particles that its destructive effect is greatly diminished; an additional percentage is broken into the form of splinters which are not destructively effective. This condition, known as lack of uniformity of fragmentation, results from the inherent lack of a uniform metallic structure throughout the body of a shell and is a necessary result of the pierce and draw method of body formation. A still further object of this invention is to provide a method of making shell forgings wherein the metal will be so manipulated as to produce a greater uniformity of structure than has hitherto been attained with the result that the finished shell will have a greater uniformity of fragmentation and consequently a higher destructive efficiency than has heretofore been possible.

These and other objects which will appear obvious to those skilled in this particular art are accomplished by means of this invention, certain steps of which are illustrated in the accompanying drawings, in which Figure 1 is a longitudinal sectional view of a tubular blank formed from metal which has been so manipulated and worked as to provide a highly uniform metallic structure throughout. Figs. 2 to 6, inclusive, are similar views showing the shell blank during different stages of its manufacture. Fig. 7 is an end view of the blank illustrated in Fig. 1, and Fig. 8 is a similar view of the partially formed blank shown in Fig. 2.

The steel from which the blank shown in Fig. 1 is produced is usually in the form of square or rectangular billets. In order to produce a blank having a thoroughly homogeneous structure so as to provide a very high uniformity of fragmentation in the completed shell the metal of the billet is so worked and manipulated in being formed into the hollow blank as to insure a uniformity of metallic structure throughout the blank. Such manipulation of the metal is

preferably obtained by first hot rolling the billets into round bars, the diameters of which will vary in accordance with the size of the blank to be produced which in turn is determined by the caliber of shell being manufactured.

The bars are then heated to a temperature of substantially 2,000° F. and are then passed through conically shaped rolls which cooperate with a revolving mandrel in simultaneously rolling the round rods and piercing the same to provide a rough tubular blank. A convenient way of piercing the solid bar and at the same time thoroughly working the metal thereof in order to produce homogeneity of structure is to provide a revolving mandrel of substantial length over which the pierced bar is rolled. The piercing of the bar is done by a blunt nosed, somewhat conically shaped plug, which is dropped in front of the mandrel as the bar enters the rolls. The mandrel pushes this plug into the end of the billet as it comes through the rolls and holds it there while the rolls force the metal over the plug and along the mandrel. The plug is not directly attached to the mandrel but floats freely as the tube is being formed. Its engagement with the mandrel causes it to rotate during the piercing action with the result that the metal of the billet is thoroughly worked or kneaded as the rough tubular blank is formed.

In this way the steel is given a highly homogeneous structure throughout, and practically all stratification of the metallic structure is eliminated. The plug being more or less floating during this step naturally seeks the center of the billet and a rough tubular blank having the desired structural characteristics referred to is formed. If desired, a small hole can be formed in the end of the billet prior to its passage through the rolls so as to permit the rotating plug to obtain an entering wedge into the billet.

The rough blank thus formed has a wavy appearance on its exterior and it is then passed through another set of rolls and over a common ball mandrel. This operation smooths out the wavy exterior of the blank and to a certain extent sizes the interior thereof. This step is preferably repeated by passing the blank through a third set of rolls and over another ball mandrel which constitutes a final sizing operation. In each of these last named steps the metal of the blank is again worked so as to increase its homogeneity of structure. The blank which still has a bright red heat is then slowly cooled until it is black.

The metal of the tubular blank so produced has had all stratification of structure eliminated by the thorough working and kneading to which it has been subjected and its structure is found to be uniform throughout.

It will also be apparent to those skilled in the

art, that the standard machinery employed in the manufacture of seamless tubing has been utilized.

When cool the blank is cut into units so as to form a hollow tubular blank 10, the length of which depends upon the size of projectile being manufactured, and this projectile blank is bored on the inside to provide a finished surface sized to the proper interior diameter, and to eliminate eccentricity. This boring can be performed on a standard machine and no special equipment is required. The bored blank is then heated to a temperature of about 1,800° F. and one end thereof is shaped to provide a flat closed end 11 and this can be done most conveniently by placing the blank in a die of the proper shape and pressing the end thereof so as to form a square based forging. The mandrel is then removed and the blank allowed to cool slowly. This operation forms the tubular blank, which was open at both ends, into a blank closed at one end having its interior cavity at the closed end the shape of the finished shell or the shape of the finished blank which has hitherto been produced by the pierce and draw method. The interior of the closed base was formerly the side wall of the hollow blank and hence the single machining operation to which the interior of the blank has been subjected provides a machined surface for the base of the forging. The operation of closing the end of the blank forces scale and other impurities 12 to the center of the closed end and it is, therefore, necessary to remove these impurities. This is accomplished by drilling or otherwise boring a hole 14 at the center of the base which is preferably conical in shape, having inwardly converging walls. The other end of the forging is then forged to form a tapered nose 13 by means of a Naze hammer after which the interior of the tapered nose is bored out to form the cylindrical surfaces 15 and 16.

As stated, the hole 14 in the base is preferably tapered and a conical plug 17 is screwed or otherwise secured in it. The forging is then placed upon a vertical mandrel with the inner end of the plug resting on the end of the mandrel. While so positioned a press is used for pressing the plug so that it spreads and completely closes the drilled hole 14 to insure a rigid connection between the plug and the base and a tight fit of the plug in the base. In view of the fact that the walls of the tapered opening 14 converge inwardly there is no danger of the plug 17 being loosened when the shell is fired from a gun, as the force of the discharge will tend to drive the plug into a tighter fitting relationship with the base of the shell.

The forging is finished by cutting threads 18 in the cylindrical surface 15 of the nose; and these are employed in securing a fuse or detonating device to the projectile. A copy

per band receiving groove 19 is cut in the outer face of the forging for the purpose of receiving the copper rifling band.

The metal from which the plug is made may be the same steel as that from which the shell forging is produced, or, if desired, it may be of softer, more easily flowing metal so as to insure a tight closing of the base when the plug is pressed therein.

10 The forging may be heat treated at any desired point in the process.

As a result of this method it is possible to produce shell forgings by means of standard machinery in vast quantities with a comparatively few men. All necessity for the special machinery required in the pierce and draw method of manufacture is eliminated and the number of men and time required to produce a given quantity is materially less. In addition to this, the saving in material is substantial.

20 Due to the thorough working to which the metal of the forging is subjected it possesses physical properties which increase its destructive effect over the shell made by the pierce and draw method because of its more homogeneous structure resulting in a greater uniformity of fragmentation upon bursting.

It will be obvious that the sequence of certain of the steps herein described may be varied as desired. For example, the plug 17 may be secured in the face 11 prior to nosing in the other end of the blank. It will be obvious that such changes may be made in the described method without departing from the spirit of this invention or the scope of the appended claims.

What I claim as new and desire to secure by Letters Patent is:

40 1. The method of making a shell forging which consists in providing a tubular blank, machining the interior of said blank, forging one end thereof so as to provide a closed, substantially flat end shell base, drilling the center of said closed end to remove oxides and porosity, shaping the other end of said blank to form a tapered nose, shaping the interior of said nose and closing the drilled opening in said base from the outside thereof.

50 2. The method of making shells which consists in machining the interior of a tubular blank to provide a predetermined interior diameter thereof, shaping one end thereof to form a flat closed shell base, drilling a tapered opening through the center of said base from the outside to the inside thereof to remove impurities, forming a tapered nose on the other end of said blank and plugging the drilled opening in said base from the outside thereof.

60 3. The method of making a shell forging which consists in providing a tubular blank, machining the interior of said blank, shaping one end thereof so as to provide a closed, substantially flat end, drilling the center of said

closed end to remove impurities therefrom and to provide a conical inwardly converging hole, tapering the other end of said blank to form a nose, enlarging the interior of said nose, inserting a plug in said hole from the outside of said flat end and pressing said plug so as to effectively close the base of the forging.

4. The method of making shells which consists in hot rolling a steel blank to form a solid rod, simultaneously rolling and piercing said rod to form a tube, and size rolling the tube so produced, cutting the tube to length, shaping one end thereof to form a cylindrical blank closed at one end, boring out the center of the closed end of said blank, securing a steel plug in the opening so formed and nosing in the opposite end of the blank.

5. The method of making shells which consists in hot rolling a steel blank to form a solid rod, piercing and rolling said rod to form a tube, shaping one end of said tube to provide a cylindrical blank closed at one end, boring out the center of the closed end of said blank, closing the opening so formed and nosing in the opposite end of the blank.

6. The method of making shells which consists in hot rolling a steel blank to form a solid bar, simultaneously rolling and piercing said bar to form a tubular blank, sizing said tube, shaping one end thereof to form a closed flat end, nosing in the opposite end of said blank and shaping the interior diameter of said nose to receive a fuse.

7. The method of making a shell forging which consists in providing a hot rolled seamless tube, machining the interior of said tube, upsetting one end thereof to provide a closed end, redrilling and plugging said closed end from the outside thereof, and forging the other end of said tube to form an open nose.

8. The method of making a shell forging which consists in providing a hot rolled seamless tube, upsetting one end thereof to provide a closed end, drilling the center of said closed end to form a tapered opening having inwardly converging walls, closing said opening by a tapered plug, compressing said plug within said opening and shaping the other end of said tube to form a tapered nose.

In testimony whereof, I have hereunto subscribed my name this 4th day of December, 1925.

GILBERT P. McNIFF.

120

125

130